

## UNITED STATES PATENT OFFICE

LESLIE BROWN, OF MIDLAND, MICHIGAN, ASSIGNOR TO THE DOW CHEMICAL COMPANY, OF MIDLAND, MICHIGAN, A CORPORATION OF MICHIGAN

## CHAPLET

No Drawing.

Application filed July 1, 1932. Serial No. 620,539.

The present invention relates to the field of art wherein magnesium is cast in cored molds; and it is a particular object of the invention to provide an improved means for maintaining dry sand cores in a substantially fixed position in a mold whereby the making of cored magnesium castings is facilitated.

The term "magnesium" is used herein and in the appended claims to mean not only elemental magnesium, but also alloys thereof wherein the magnesium content predominates.

I have found that the difficulties inhering to prior processes of making cored magnesium castings wherein chaplets are employed for holding the core in position may be overcome by using a chaplet comprising cadmium.

To the accomplishment of the foregoing and related ends, the invention, then, consists of the steps and product hereinafter fully described and particularly pointed out in the claims, the following description setting forth in detail one mode of carrying out the invention, such disclosed mode illustrating, however, but one of the various ways in which the principle of the invention may be used.

In the casting of magnesium it has been general practice to avoid insofar as possible the use of chaplets for holding a dry sand core in position, due to the numerous disadvantages attaching to such mode of procedure. For instance, if the chaplets were made of magnesium or aluminum, it was found that, owing to the nearly equal melting points of the chaplet and magnesium and to the presence of an oxide film usually found on chaplets consisting of magnesium, such chaplets did not fuse satisfactorily during the pouring operation and that a poor casting was obtained. Various low melting metals e. g. tin, bismuth, etc., and alloys thereof, have been proposed and tried as chaplets, but all such as have been suggested possess the disadvantage of forming an alloy between the metal of the chaplet and the magnesium of such constitution that a brittle zone results in the finished casting.

In making magnesium castings it has, therefore, been established practice to avoid the use of chaplets as by suspending the cores

from the top of the mold. However, such procedure can not always be employed without unduly complicating the mold and further, when used, is often excessively time-consuming and expensive. By using chaplets consisting of cadmium I have been able to support dry sand cores in molds wherein the thickness of finished casting approximated one eighth of one inch, and have determined that such practice results in substantially perfect fusion between the chaplet and the magnesium, whereby a finished casting of excellent quality free from brittleness is obtained. In certain instances, such as in supporting a core in a mold wherebetween an extremely thin section is to be cast, it may be found desirable to employ an alloy of cadmium with relatively small amounts of other suitable metals adapted to depress the melting point of the cadmium, e. g. zinc, tin, lead, etc., whereby a chaplet having a fusing point lower than that of pure cadmium can be obtained.

In supporting cores in molds wherein the thickness of the section to be cast is somewhat greater, e. g. one to two inches or more, I have found it advantageous to use a chaplet consisting of cadmium alloyed with an amount of magnesium sufficient to elevate the melting point of the chaplet to a temperature such that the chaplet does not lose its strength by fusion with the magnesium being poured into the mold before performing its function of supporting the core. It is evident that the composition of the chaplet may be varied over a wide range, since cadmium and magnesium alloy perfectly in all proportions, and further it is evident that a chaplet of any desired melting point in the range between the melting points of cadmium and magnesium may be readily obtained, or that small amounts of zinc, tin, etc., may be incorporated with the cadmium-magnesium in order to improve the properties thereof.

Manifestly, my chaplet may be constructed in any suitable form, e. g. double head with round or square plates, double head water-back, saddleback or bridge, curved, ferrule, etc., without departing from the spirit of my invention.

Other modes of applying the principle of my invention may be employed instead of those explained, change being made as regards the steps and means herein disclosed, 5 provided those stated by any of the following claims or their equivalent be employed.

I therefore particularly point out and distinctly claim as my invention:—

1. In casting magnesium the method of 10 maintaining a dry sand core in a substantially fixed position in a mold which comprises interposing between the core and the mold a chaplet comprising cadmium.
2. In casting magnesium the method of 15 maintaining a dry sand core in a substantially fixed position in a mold which comprises interposing between the core and the mold a chaplet comprising cadmium having alloyed therewith magnesium.
- 20 3. In casting magnesium the method of maintaining a dry sand core in a substantially fixed position in a mold which comprises interposing between the core and the mold a chaplet consisting of cadmium having alloyed therewith a relatively small amount of a metal from the class consisting of zinc, lead, and tin.
- 25 4. A chaplet for use in maintaining a dry sand core in a substantially fixed position in a mold while casting magnesium in the said mold composed predominantly of cadmium.
- 30 5. A chaplet for use in maintaining a dry sand core in a substantially fixed position in a mold while casting magnesium in the said mold consisting of cadmium having alloyed therewith magnesium.
- 35 6. A chaplet for use in maintaining a dry sand core in a substantially fixed position in a mold while casting magnesium in the said mold consisting of cadmium having alloyed therewith a relatively small amount of a metal from the class consisting of zinc, lead, and tin.

Signed by me this 28th day of June, 1932.

45 LESLIE BROWN.